

Aug. 18, 1953.

H. A. BRUSON

2,649,356

METHOD OF HANDLING POLYMERIC COMPOSITIONS

Filed Oct. 13, 1950



INVENTOR  
HERMAN A. BRUSON  
BY Philip J. Caneva  
ATTORNEY

## UNITED STATES PATENT OFFICE

2,649,356

## METHOD OF HANDLING POLYMERIC COMPOSITIONS

Herman A. Bruson, Shaker Heights, Ohio, assignor to Industrial Rayon Corporation, Cleveland, Ohio, a corporation of Delaware

Application October 13, 1950, Serial No. 190,056

4 Claims. (Cl. 18—54)

1

This invention relates to the handling of ethylene carbonate solutions of acrylonitrile polymers. More particularly, it relates to a spin-solution handling process which permits the reclamation and recovery of such polymeric solutions in a colorless condition and thus capable of being re-used to form acceptable fibers, filaments, films and the like, hereinafter referred to as fibers.

Both prior to and during the extrusion of such spinning solutions into a coagulating medium, it is often found necessary to interrupt the coagulation action and to set aside and collect the uncoagulated spinning solution. There are various reasons for these interruptions such as, for example, the following: (a) prior to extrusion it is the usual practice to pump substantial quantities of the spinning solution through the spinneret until all of the impurities in the lines are removed and other conditions such as temperature, viscosity, etc., have attained the desired normalcy; (b) to adjust the spinning differences that may exist from batch to batch of solution and from one spinning position to the next; (c) broken filaments or fibers; (d) to store excess quantities of prepared spinning solution for future use. Such collected or stored spinning solutions are capable of being re-used to form acceptable fibers provided that efficient and non-color-forming reclamation methods are used.

The nature of the spinning solution is the principal source of the handling and reclamation difficulties referred to above. When warm, the solution is a viscous sticky syrup which sets to a rubbery, adherent plastic jelly at ordinary room temperature. It is very difficult to handle in that it sticks tenaciously to any surface, and therefore, cannot readily be removed from receptacles or containers in which it is collected or temporarily stored. Furthermore, the use of heat for prolonged periods to remove such adherent material from receptacles, causes undesirable darkening of the polymeric material rendering it unsuitable for the spinning of fibers.

In accordance with the process of the present invention, not only can the collected spinning solution be reclaimed and re-used to form colorless fibers, but in addition, the containers for collecting or storing the solution can also be re-used with practically no cleaning operation. In accordance with the present invention, an ethylene carbonate solution of certain acrylonitrile polymers which is being extruded from a heated system through a spinneret while in a fluid state is collected in a container, the walls of which slope inwardly toward the bottom thereof, and the collected material thereafter cooled to a tempera-

2

ture below about 20° C. The solidified material is removed from the container and later returned to the heated system from which it can be extruded to form fibers. The polymeric solutions employed in accordance with the present invention comprise ethylene carbonate and an acrylonitrile polymer dissolved therein having in the polymer molecule at least about 80% by weight acrylonitrile. The spinning solution contains between about 15 and 25% by weight of the polymeric material.

The spinning solution which has been cooled until solidified is transformed into a hard, tough, wax-like solid. This occurs at temperatures below about 20° C. and advantageously, within the range of about +15° to —15° C., and preferably, between about +5° and —5° C. During this solidification, a certain amount of contraction and shrinkage in the volume of the material occurs, and its adherence to smooth surfaces such as metal surfaces practically completely disappears. The solid bar of wax-like material can then be easily lifted or dumped out of the container and added to new batches of spinning solution as desired.

The containers used for the purposes of this invention may be made of any smooth-surfaced rigid material and of a wide variety of sizes depending upon the quantity desired to be collected or stored. Particular advantages, however, are derived with containers made from metal sheets, e. g., of stainless steel, aluminum, galvanized iron, etc. Preferably, the container and particularly the opening thereof should be of such a shape as to permit the easy removal of the solidified material. As stated above, the walls of the container slope inwardly toward the bottom thereof, and advantageously, may be shaped like a V or U, so that the resulting waxy bar easily falls out when the container is turned upside down and tapped.

The condition of the container after the removal of the waxy solidified material is such that it may be re-used, i. e., refilled, immediately and repeatedly without performing any polymer-cleaning operation on the container. Where hundreds of spinning positions of spinnerets are to be serviced each with an individual container, it is apparent that the process of the present invention provides substantial savings not only in initial equipment cost but also in material cost and in maintenance expenses. In addition, of course, it provides for the reclamation or storage, or both, of spinning solution material in colorless spinnable condition.

This invention will be more fully described by

the following example, although it is understood that the invention is not intended to be limited by this example. In this example "parts" and "percent" of materials is intended to mean parts and percent by weight.

*Example*

20 parts of polyacrylonitrile (average molecular weight about 42,000) is dissolved in 80 parts ethylene carbonate by mixing and heating to about 100° C. This solution after filtering and deaerating, under vacuum, is heated to 120° C. and extruded through a spinneret having 40 holes (.003 inch diameter). Prior to starting the actual extrusion into the coagulating bath, the extruded spinning solution is collected in a stainless steel container having walls sloping inwardly to the bottom thereof, i. e., U shape. This extrusion and collection is permitted to continue at one spinning position until about 1000 grams of material is collected and substantially all of the impurities in the lines are removed and the temperature and viscosity of the solution have attained the desired normalcy. Thereafter, the spinneret is plunged into the bath liquid and the extruded spinning solution coagulated in a bath consisting of 80 parts triethylene glycol and 20 parts ethylene carbonate.

The 1000 gram portion of the spinning solution collected in the container is placed in a refrigerator maintained at 0° C. After one hour, the container is removed, the spinning solution having completely solidified into a shrunken waxy solid. The container is then inverted and the solidified material is caused to fall therefrom by tapping the bottom of the container. The bar of solidified material is then added to a quantity of heated spinning solution and caused to dissolve therein. The resulting blended spinning solution is extruded and coagulated in the coagulating bath described above. The emptied stainless steel container is clean and free from particles of polymeric material. The container is then re-used for the same purpose and without any cleaning operation. The bath temperature is maintained at 130° C. while the coagulated filaments are drawn through the bath for 30 inches of bath travel and then collected on bobbins rotating at a peripheral speed of about 44 meters per minute. The yarn is then washed, stretched and relaxed to produce a final product which is light-colored and of uniform quality having a soft, silky feel, a denier of about 94, a breaking tenacity of about 4.4 grams per denier, and a breaking elongation of about 18%.

As previously stated, the acrylonitrile content of the polymer in the spinning solution is at least 80%, and particular advantages are derived with copolymers having a greater percentage of acrylonitrile. Among the fiber-forming copolymers which may be employed with advantage in accordance with the process of this invention may be mentioned copolymers of acrylonitrile with the following monomeric compounds: vinyl esters (vinyl acetate, vinyl formate, vinyl benzoate), vinyl ethers, and vinyl ketones; acrylic acid and its esters and amides; methacrylic acid and its esters, amides, and nitrile; maleic, itaconic, fumaric, crotonic acids and their esters, amides and nitriles; allyl alcohol and its esters; styrene and nuclear substituted styrenes, e. g. chloro- and dichloro styrene; halogenated monoethylenic compounds such as vinyl chloride, vinyl fluoride, and vinylidene chloride; N-vinyl compounds such as N-vinyl pyrrolidone, N-vinyl suc-

cinimide, N-vinyl carbazole, 2- and 4-vinyl pyridine; and the like.

The acrylonitrile polymers and copolymers may be prepared by any suitable polymerization method such as, for example, the ammonium persulfate catalyzed polymerization of monomer or monomers dissolved or emulsified in water. Molecular weights of these polymers and copolymers are preferably within the range of 10,000 and 250,000, or even higher, although polymers having molecular weights between 30,000 and 150,000 may be used with particular advantage in the production of fibers.

In general, the spinning solutions may be prepared by heating a mixture of the finely divided acrylonitrile polymer or copolymer with the ethylene carbonate solvent until the polymer is dissolved. Advantageously, the spinning solution may be maintained, prior to extrusion, at temperatures from about 80° to 150° C., and preferably between about 110° and 130° C.

The cooled and solidified material may be stored as such in the containers, or more advantageously may be removed and re-used directly in preparing new batches of spinning solution or may be blended with solutions undergoing spinning and coagulation. If desired, the solidified material may be converted into smaller particles to facilitate the dissolving thereof. Under certain conditions, it may be desirable to store the solidified material for future use either in bar form or in a broken form.

I claim:

1. A process for handling and reclaiming an ethylene carbonate spinning solution of an acrylonitrile polymer which is being extruded from a heated system through a spinneret while in a fluid state, the steps comprising collecting said material in a container; cooling said material in said container to a temperature below about 20° C.; removing the resulting cooled and solidified material from said container; returning said solidified material to said heated system; re-using said container for the collection of additional quantities of said spinning solution, without performing any polymer cleaning operation on said emptied container between said emptying and refilling operations; said solution comprising ethylene carbonate and an acrylonitrile polymer dissolved therein having in the polymer molecule at least about 80% by weight acrylonitrile; said spinning solution containing between about 15 and 25% by weight of polymeric material; the walls of said container sloping inwardly toward the bottom thereof.

2. A process for handling and reclaiming an ethylene carbonate spinning solution of an acrylonitrile polymer which is being extruded from a heated system through a spinneret while in a fluid state, the steps comprising, collecting said extruded material in a container; cooling said extruded material in said container to a temperature between about +15° and -15° C.; removing the resulting cooled and solidified material from said container; returning said solidified material to said heated system and spinning fibers therefrom; re-using said container for the collection of additional quantities of said spinning solution, without performing any polymer cleaning operation on said emptied container between said emptying and refilling operations; said solution comprising ethylene carbonate and an acrylonitrile polymer dissolved therein having in the polymer molecule at least about 80% by weight acrylonitrile; said spinning solution

containing between about 15 and 25% by weight of polymeric material; the walls of said container sloping inwardly toward the bottom thereof.

3. A process for handling and reclaiming an ethylene carbonate spinning solution of an acrylonitrile polymer which is being extruded from a heated system through a spinneret while in a fluid state, the steps comprising, collecting said extruded material in a metal container; cooling and solidifying said extruded material in said container to a temperature between about +15° and -15° C.; inverting said cooled container so as to cause said solidified material to fall therefrom; returning said solidified material to said heated system and spinning fibers therefrom; re-using said container for the collection of addi- 10 15

tional quantities of said spinning solution, without performing any polymer cleaning operation on said emptied container between said emptying and refilling operations; said solution comprising ethylene carbonate and an acrylonitrile polymer dissolved therein having in the polymer molecule at least about 80% by weight acrylonitrile; said spinning solution containing between about 15 and 25% by weight of polymeric material; the walls of said container sloping inwardly toward the bottom thereof.

4. A process according to claim 3 in which the container is a stainless steel container.

HERMAN A. BRUSON.

No references cited.